

Jan. 11, 1938.

A. J. WEINIG

2,105,294

TEMPERATURE CONTROL IN A FLOTATION PROCESS

Filed Dec. 1, 1934



Fig. 2

Fig. 3

Fig. 4



Fig. 5

Fig. 1



INVENTOR.

A. J. WEINIG

BY

  
ATTORNEY.

## UNITED STATES PATENT OFFICE

2,105,294

## TEMPERATURE CONTROL IN A FLOTATION PROCESS

Arthur J. Weinig, Golden, Colo., assignor to  
 Potash Company of America, Denver, Colo., a  
 corporation of Colorado

Application December 1, 1934, Serial No. 755,576

23 Claims. (Cl. 209—167)

This invention relates to improvements in the so-called flotation process for the separation of minerals in liquid suspension, and its primary object is to promote and expedite the separative 5 action, by temperature regulation at one or more stages of the process.

While the invention may be applied to the treatment of different ores, it is particularly adapted for use in the concentration of ores containing minerals of widely differing solubility characteristics, and it is another object of the invention to increase the differentiating effect of flotation reagents upon minerals in suspension in a flotation process, by maintaining a temperature condition under which the differential action of the reagents upon the minerals is accentuated to a degree conducive toward effecting a substantially clean separation of one mineral from another mineral or from foreign matter 20 with which it is associated in the natural formation of the ore.

It is customary in the flotation process to produce the required aeration of the material by mechanical agitation, and a further object of 25 the invention may be found in the provision of a cooling influence which counteracts the increase in temperature incident to the agitative action upon the material.

The invention is of especial value in a process 30 of separating sodium chloride or halite and potassium chloride or sylvite by flotation and the following description will be made with reference to the application of the invention to ores of this particular character.

35 The solubility of both halite and sylvite is comparatively high and the degree of solubility of the sylvite is considerably higher than that of the halite. It follows that under temperature variations in a pulp in which these minerals are 40 suspended, the solubility of the halite changes very slowly in comparison with that of the sylvite.

Since the flotation process is dependent upon 45 the differential action of reagents upon a mineral to be separated, by coating the particles thereof with a substance which causes the same to adhere to rising air-bubbles, the process is essentially a surface phenomenon. Minerals or other matter in the ore which are to be separated 50 from the rising mineral either are not

coated or are differentially coated, so that only those particles coated with a substance which causes them to adhere to the rising air-bubbles will rise to the surface of the liquid mass, to be recovered by overflow or the like.

It follows that an ideal situation in the flotation process will be that in which all the halite in the material is constantly present in solid form, and the proper differential action on the surface of its particles will be effectively produced and maintained throughout the process.

The sylvite owing to its high rate of solubility with temperature increase, is more affected by temperature variations than the halite. Normally neither mineral will, by itself, collect in the 15 froth of the flotation cell and to produce the most stable flotation, the halite surfaces must be subjected to the reaction of the reagent while the sylvite surfaces may be differentially reacted upon or remain comparatively in their natural 20 condition. Temperature conditions in the material are thus an influence which to a large extent controls the separative action.

If by the mechanical agitation of the material or by other causes such as climatic changes, the 25 temperature of the material increases, part of the metallic particles are brought into solution or the delicate flotation surfaces are dissolved off. Also varying temperatures at different stages of the process will cause erratic flotation.

30 With the above facts in mind it will be seen that by maintaining an even temperature throughout the material under treatment, at which substantially all the material is maintained in suspension, or prevented from going 35 into solution, a clean separation of the sylvite from the halite may be effected.

At a lowered temperature, sylvite will deposit out of solution onto the existing sylvite surfaces, and be recovered in the potassium chloride concentration, thereby promoting its separation from the sodium chloride rising to the surface.

If at the higher temperature coated halite surfaces are covered by other halite deposited out of solution, additional flotation agent can be used 45 to maintain the flotation surface, particularly at the tail end of the flotation period.

Ordinarily a reduction of temperature is required to produce the desired result, and this may be accomplished through the medium of a 50

jacket around the flotation cell, or a coil within the same, through which a cooling fluid is circulated. It is also possible however, that due to climatic conditions or other factors, an increase in temperature is necessary to bring the material to or near the ideal condition above stated, and it is to be understood that by referring to temperature-regulation, both conditions are included.

10 In the accompanying drawing,

Figure 1 is a diagram showing the comparative solubility characteristics of the potassium chloride and sodium chloride in an aqueous pulp of the ore,

15 Figure 2 is an outline of a flotation cell to which the invention is applied.

Figure 3 is a similar view showing a different method of temperature-regulation.

20 Figure 4 is a diagrammatic view of a system for recovering the sylvite in a flotation process, showing the application of the invention at different stages thereof, and

25 Figure 5 is a modification of the system depicted in Figure 4.

25 In the treatment of halite-sylvite ores by flotation, the ore in a finely-divided condition, is mixed in a saturated solution of the minerals, in a flotation vessel of conventional form. In this cell the material is mechanically agitated and aerated by one or more rotating propellers, and it is at the same time subjected to the influence of suitable flotation agents.

30 In accordance with the present invention, the material in the cell is at the same time cooled to an even temperature of predetermined degree by the use of a jacket around the vessel or a coil within the same through which a cooling fluid, either liquid or gaseous, is circulated. If as stated hereinbefore, it is required to increase 35 the temperature of the material, a heating fluid is, of course, substituted for the cooling fluid.

35 Referring further to the drawing, the material is fed into the flotation vessel 5 at 6, the froth with the mineral entrapped therein, is discharged 40 by overflow as at 7, and matter other than that rising to the surface is discharged at the bottom of the vessel as at 8. The pulp in the vessel is aerated and agitated by rotating propellers as shown at 9. In Figure 2, a cooling fluid entering 45 at 10 passes through a jacket 12 around the vessel, and leaves the jacket at 13 after having lowered the temperature of the material inside the vessel to a predetermined degree.

50 In Figure 3, a coil 14 inside the vessel is substituted for the jacket.

55 In Figures 4 and 5 is shown a system by which the froth delivered from the flotation vessel is treated under temperature regulation, to recover sylvite which may have escaped with the halite, 60 after which the halite is recovered from the brine solution and the latter returned to the flotation vessel for reuse.

65 Referring first to Figure 4, the overflow of the flotation vessel passes in the direction of the line 15 to a vessel 16, containing an agitator 17. In this vessel the sodium chloride or halite froth is heated through the medium of a coil 18, causing any sylvite which escaped with the halite due to 70 attachments or other causes, to dissolve. The warmed pulp then overflows as at 19 into a thickener 20 where the sylvite-depleted halite settles out and the solution returns in the direction 21 to the head or feed end of the flotation vessel.

75 Excess sylvite in solution, will be deposited out of the solution by the cooling influence in the flotation vessel, to be recovered with the sylvite concentrate at 8.

In Figure 5, the heating fluid enters the coil 18 5 of the agitator 16 from a compressor 22, and after having heated the material in the agitator passes in a cooled condition, past an expansion valve 23 to the coil 14 or jacket 12 of the flotation vessel. Heating coils 24 in the agitator provide additional heat to balance radiation losses 10 and heat loss with halite waste.

While in the treatment of ores in accordance with the invention, the critical temperature at which the material is maintained must necessarily vary in accordance with varying conditions, it has been found that in the flotation of potassium chloride ores, a temperature of approximately sixteen degrees centigrade in the flotation vessel has produced satisfactory results, 15 in the presence of a reagent composed of a brine-soluble fatty acid and a brine-soluble metallic cation, which has been made the subject of an application for patent, separate from the present one, namely, Serial No. 755,577, filed December 25 1, 1934, for Flotation process. My co-pending applications, Serial No. 7,219, filed February 19, 1935, for Concentration process, Serial No. 11,059, filed March 14, 1935, for Flotation process and reagent, and 28,983, filed June 28, 1935, also disclose other reagents and treatments well suited for use in the froth flotation of these ores. Subject matter disclosed but not claimed herein have been claimed in the aforementioned applications. 30

It is to be understood that the liquid phase of the treatment is a saturated solution of sodium chloride and potassium chloride, and the solubilities of halite and sylvite in this solution have been illustrated in Figure 1. The upright column of figures represents grams of KCl or NaCl per 100 grams of water and the column of figures extending along the bottom of the chart represents temperature in degrees centigrade.

35 The solubility characteristics of these minerals in a solution of the same is tabulated on page 77 45 of "Fortschriften in Kali-Industrie", by Dr. C. Hermann, Berlin, published by Theodore Steinkopff, Dresden and Leipzig, 1927, as follows:—

Erlösen 100 teile, Wasser bei

50

| Tempera-<br>ture °C. | KCl  | NaCl |
|----------------------|------|------|
| 10                   | 12.5 | 29.7 |
| 20                   | 14.7 | 29.2 |
| 30                   | 17.2 | 28.7 |
| 40                   | 19.5 | 28.2 |
| 50                   | 22.0 | 27.5 |
| 60                   | 24.6 | 27.2 |
| 70                   | 27.3 | 26.8 |
| 80                   | 30.0 | 26.4 |
| 90                   | 32.9 | 26.1 |
| 100                  | 35.9 | 25.8 |

55

60

65

70

The foregoing figures are true, only when there are ample quantities of NaCl and KCl in the solid phase in contact with the liquid phase to permit the latter to become fully saturated with respect to both salts. When the liquid phase is not in contact with a sufficient quantity of the solid phase of one of the salts, the equilibria above noted does not exist.

To permit a complete comprehension of solubility characteristics of the pulp, treated by the present process, the following chart illustrates the equilibria of the system when there is a de- 75

iciency in the amount of either of the salts, in the solid phase; in the temperature of the solution and its solid constituent below the said selected temperature.

5 **Equilibria for the system KCl—NaCl—H<sub>2</sub>O**  
(Temperature degrees Fahrenheit)

| KCl in brine |              | 40                                           | 50   | 60   | 70   | 80   | 90   | 100  | 110  | 120  | 130  | 140  | 150  |      |
|--------------|--------------|----------------------------------------------|------|------|------|------|------|------|------|------|------|------|------|------|
| Gr.<br>litre | Per<br>cent. | Per cent. sodium chloride in saturated brine |      |      |      |      |      |      |      |      |      |      |      |      |
| 10           | 97           | 7.9                                          | 21.2 | 21.4 | 21.5 | 21.7 | 21.9 | 22.1 | 22.2 | 22.4 | 22.6 | 22.7 | 22.9 | 23.1 |
|              | 108          | 8.7                                          | 19.8 | 20.9 | 21.1 | 21.2 | 21.4 | 21.6 | 21.8 | 21.9 | 22.1 | 22.3 | 22.4 | 22.6 |
|              | 118          | 9.6                                          | 18.4 | 19.5 | 20.6 | 20.8 | 20.9 | 21.1 | 21.3 | 21.5 | 21.6 | 21.8 | 22.0 | 22.1 |
|              | 130          | 10.4                                         | 16.9 | 18.0 | 19.1 | 20.2 | 20.4 | 20.5 | 20.7 | 20.9 | 21.1 | 21.2 | 21.4 | 21.6 |
|              | 140          | 11.3                                         | 15.5 | 16.6 | 17.7 | 18.8 | 19.9 | 20.1 | 20.2 | 20.4 | 20.6 | 20.8 | 20.9 | 21.1 |
| 15           | 151          | 12.2                                         | 14.0 | 15.1 | 16.2 | 17.3 | 18.4 | 19.5 | 19.7 | 19.9 | 20.0 | 20.2 | 20.4 | 20.5 |
|              | 162          | 13.0                                         | 12.6 | 13.7 | 14.8 | 15.9 | 17.0 | 18.1 | 19.2 | 19.4 | 19.5 | 19.7 | 19.9 | 20.1 |
|              | 172          | 13.9                                         | 11.2 | 12.3 | 13.4 | 14.5 | 15.6 | 16.7 | 17.8 | 18.9 | 19.1 | 19.2 | 19.4 | 19.6 |
|              | 183          | 14.7                                         | 9.7  | 10.8 | 11.9 | 13.0 | 14.1 | 15.2 | 16.3 | 17.4 | 18.5 | 18.6 | 18.7 | 19.0 |
|              | 194          | 15.5                                         | 8.3  | 9.4  | 10.5 | 11.6 | 12.7 | 13.8 | 14.7 | 16.0 | 17.1 | 18.2 | 18.4 | 18.5 |
| 20           | 205          | 16.4                                         | 6.9  | 8.0  | 9.1  | 10.2 | 11.3 | 12.4 | 13.5 | 14.6 | 15.7 | 16.8 | 17.9 | 18.1 |
|              | 216          | 17.3                                         | 5.4  | 6.5  | 7.6  | 8.7  | 9.8  | 10.9 | 12.0 | 13.1 | 14.3 | 15.4 | 16.5 | 17.6 |

The boxed figures are from equation (B) see below.

$$\% \text{NaCl} = 30.3 - 1.7K + 1.1T < 22.6 - .033T < 25.3 - .6K + .017T$$

(A) (B) (C)

25 Values to the left of boxed figures Values to right of boxed figures

- (A) Equation when deficiency exists in the NaCl solid phase.  
(B) Equation when no deficiency exists in the solid phases.  
(C) Equation when deficiency exists in the KCl solid phase.

K=% KCl in brine  
T=Temperature Fahrenheit degrees

30 Examples of the application of the foregoing to the flotation treatment will serve to illustrate the importance of the temperature control of the present invention.

35 If, on heating a flotation pulp or concentrate containing little KCl with much NaCl in the solid phases, all the KCl solids will pass over to the liquid phase in the solution at 100° F. for example, and the liquid phase will then show 13.0% KCl and 19.2% NaCl.

40 With continued heating to 150° F., for example, no more KCl can enter the liquid phase, due to the absence of KCl solids, and additional NaCl will then enter the liquid phase, with the result that analysis of the solution will disclose 13.0% KCl and 20.1% NaCl at this temperature.

45 Likewise, on cooling this solution back to 100° F., NaCl alone will crystallize out and on further cooling below 100° F., KCl will crystallize out of solution while NaCl will again go into solution. For example, if cooling is continued to 70° F. the solution or liquid phase will show 20.2% NaCl and 10.4% KCl.

50 Thus it is apparent, that a flotation treatment of these ores in which temperature control is not practiced would not be entirely efficient due to solubility losses, and a clean separation in the various treatments will not be attained unless controlled temperatures are employed. This is extremely important when the pulps which have been separated by flotation individually, receive heating or cooling treatments.

55 What I claim and desire to secure by Letters Patent is:

60 1. A selective flotation process for separating soluble constituents of an ore having different solubility characteristics that vary under temperature variations, which comprises introducing a halite-sylvite ore into a saturated solution of the same to form a pulp at a selected temperature, subjecting the pulp to a froth flotation process, including the use of a reagent having a selective affinity for one of said constituents, and in the remaining saturated solution inducing a crystallization of its other soluble constituent by lower-

30 2. A selective flotation process for separating soluble constituents of an ore having different solubility characteristics that vary under temperature variations, which comprises introducing a halite-sylvite ore into a saturated solution of the same to form a pulp at a selected temperature, subjecting the pulp to a froth flotation process, including the use of a reagent having a selective affinity for one of said constituents, and separating the said constituents by inducing a crystallization of one of the soluble constituents and dissolution of the other soluble constituent of the saturated solution by raising its temperature above that of the selected temperature.

35 3. A selective flotation process for separating soluble constituents of an ore having different solubility characteristics that vary under temperature variations, which comprises introducing a halite-sylvite ore into a saturated solution of the same to form a pulp, subjecting the pulp to a froth flotation process, including the use of a reagent having a selective affinity for sodium chloride, and maintaining the pulp during said treatment at a substantially uniform temperature at which the soluble halite particles will not go into solution in the pulp.

40 4. A selective flotation process for separating soluble constituents of an ore having different solubility characteristics that vary under temperature variations, which comprises introducing a halite-sylvite ore into a saturated solution of the same to form a pulp, subjecting the pulp to a froth flotation process, including the use of a reagent having a selective affinity for one of said constituents, and maintaining the pulp during the said treatment at a temperature at which the soluble sylvite particles will not go into solution in the pulp.

45 5. A selective flotation process for separating soluble constituents of an ore having different solubility characteristics that vary under temperature variations, which comprises introducing a halite-sylvite ore into a saturated solution of the same to form a pulp, subjecting the pulp to froth flotation, including the use of a reagent

- having a selective affinity for the halite and gangue constituents, maintaining an operating temperature during flotation at which soluble halite particles in the pulp will not go into solution, then raising the temperature of froth product of flotation to dissolve any sylvite in the same, and then separating the solids from the solution.
6. A selective flotation process for separating soluble constituents of an ore having different solubility characteristics that vary under temperature variations, which comprises introducing a halite-sylvite ore into a saturated solution of the same to form a pulp, subjecting the pulp to froth flotation, including the use of a reagent having a selective affinity for the halite and gangue constituents, subjecting the pulp during the flotation treatment to a cooling influence sufficient to counteract the rise in temperature due to the froth flotation treatment, recovering sylvite from the froth product of flotation by heating said product sufficiently to bring sylvite particles into solution, then removing the solid constituents from the solution, and finally re-turning the solution containing the dissolved sylvite for re-use in the flotation treatment.
7. A selective flotation process for separating soluble constituents of an ore having different solubility characteristics that vary under temperature variations, which comprises introducing a halite-sylvite ore into a saturated solution of the same to form a pulp, subjecting the pulp to froth flotation, including the use of a reagent having a selective affinity for the halite and gangue constituents, subjecting the pulp during the flotation treatment to a cooling influence sufficient to counteract any rise in temperature incident to the froth flotation treatment, recovering sylvite from the froth product of flotation by passing the same into solution in a heated fluid, then removing the solid constituents from the solution, then returning the solution containing the dissolved sylvite for re-use in the flotation action, cooling said heated fluid, and utilizing it to cool the material during the flotation action.
8. A selective flotation process for separating soluble constituents of an ore having different solubility characteristics that vary under temperature variations, which comprises introducing a halite-sylvite ore into a saturated solution of the same to form a pulp, subjecting the pulp to froth flotation including the use of a reagent having a selective affinity for the halite and gangue constituents, whereby a froth containing halite and some sylvite is produced, then agitating the froth product of flotation while raising its temperature sufficient to bring the sylvite into solution but not high enough to bring the halite into solution, removing the solution from the undissolved constituents of the froth product, and returning said solution for reuse in the flotation treatment.
9. In a method of froth flotation separation of two soluble minerals, one of which is soluble at a lower temperature than the other, the steps of entering a mixture of sylvinite ore into a saturated solution of the ore to form a pulp, subjecting the pulp to a froth flotation treatment in the presence of a flotation reagent having a selective affinity for halite constituents whereby a froth overflow product is formed, maintaining a temperature during the flotation treatment below that at which sylvite particles will be dissolved, then subjecting the froth overflow prod-
- uct to a temperature high enough to cause particles of sylvite to pass into solution and below that at which the halite particles will pass into solution, and subjecting the said overflow product to a separation treatment for the removal of solids from the solution.
10. In a flotation process for the treatment of ores containing potassium chloride and sodium chloride, the steps of suspending said particles in a saturated solution of the ore, treating said particles to froth flotation, and maintaining a substantially uniform temperature during the froth flotation treatment, said temperature being one at which the liquid phase will neither deposit out of solution nor dissolve one of said soluble ore constituents.
11. In a flotation process for the treatment of ores containing potassium chloride and sodium chloride suspended in a saturated solution of the ore inclusive of a froth flotation treatment, the step of maintaining a substantially uniform temperature during the froth flotation treatment, said temperature being one at which the liquid phase will neither deposit out of solution nor dissolve either of said soluble ore constituents.
12. In a flotation process for the treatment of sylvinite ores, the steps of raising the temperature of a product of flotation containing solid phases of potassium chloride and other ore constituents thereby causing the said potassium chloride in the solid phase to enter into solution in its liquid phase, then separating the liquid from the solid phase, and then cooling the separated liquid phase so as to cause potassium chloride solids to separate therefrom.
13. In a flotation process for the treatment of sylvinite ores, the steps of raising the temperature of a product of flotation containing solid phases of potassium chloride and other ore constituents thereby causing the said potassium chloride in the solid phase to enter into solution in its liquid phase, separating the liquid from the solid phase, entering the separated liquid phase into pulp which has been enriched in potassium chloride in the solid phase, and then cooling the mixture thereby causing potassium chloride to deposit out of its liquid phase into its solid phase.
14. In a flotation process for the treatment of sylvinite ores by suspension in a pulp at a predetermined temperature and treatment to froth flotation, the step of raising the temperature of the froth product of flotation to cause potassium chloride in the solid phase in said product to enter into solution in the liquid phase.
15. The process of treating sylvinite ores, which comprises introducing sylvinite ore in finely-divided condition into a saturated solution of the ore to form a pulp, subjecting the undissolved sodium chloride particles of the pulp to the action of a froth flotation reagent having a selective affinity therefor, removing the resulting froth carrying sodium chloride, subjecting said froth to heat and agitation, whereby any potassium chloride particles associated with the sodium chloride particles will be dissolved, and then separating the undissolved sodium chloride particles from the solution.
16. In a process of treating sylvinite ores, the steps of subjecting such sylvinite ores in a saturated solution thereof to a flotation treatment, subjecting the froth concentrate of flotation to agitation at a controlled temperature to effect separation between the undissolved mineral par-

ticles in the froth by dissolving one of the constituents into the solution, removing the separated mineral particles, and returning the solution to the process.

5 17. In a process of treating sylvinitic ores, the steps of subjecting such ores in a saturated solution of the ores to a flotation treatment in the presence of a reagent having a selective affinity for sodium chloride, maintaining the temperature of the flotation pulp substantially uniform during the flotation operation, and then raising the temperature of the froth concentrate of the flotation operation.

15 18. In a process of treating sylvinitic ores, the steps of subjecting such ores in a saturated solution of the ores to a flotation treatment in the presence of a reagent having a selective affinity for sodium chloride, maintaining the temperature of the flotation pulp substantially uniform during the flotation operation, and then raising the temperature of the froth concentrate of the flotation operation, whereby any potassium chloride associated with sodium chloride in the froth is dissolved and sodium chloride passes out of solution, separating sodium chloride solids from the solution, and then lowering the temperature of the solution to cause potassium chloride to pass out of solution.

20 19. In a flotation process for the treatment of sylvinitic ores, by suspension in a pulp at a predetermined temperature and treatment to froth flotation, the step of raising the temperature of the froth product of flotation to cause sodium chloride in the liquid phase in said product to deposit out of solution into solid form.

25 20. A cyclic froth flotation process for the treatment of sylvinitic ore, which comprises subjecting the ore to froth flotation in a pulp composed of solid phases of the ore suspended in a liquid phase which is a saturated solution of the ore, returning the liquid phase to the process for reuse in flotation at controlled temperature, and

regulating said flotation temperature by subjecting said liquid phase to an artificial withdrawal of heat compensating for the temperature increase generated in the prior cyclic movement.

21. In a cyclic froth flotation process for the treatment of sylvinitic ore, subjecting the ore to froth flotation at a substantially uniform temperature in a pulp composed of solid phases of the ore suspended in a liquid phase which is a saturated solution of the ore, returning the liquid phase to the process for reuse in flotation at said controlled temperature, and successively raising and lowering the temperature of the solution between repetitions of flotation to crystallize constituents of the saturated solution separately at different stages of the cycle.

25 22. In a cyclic froth flotation process for the treatment of sylvinitic ore, subjecting the ore to froth flotation at a substantially uniform temperature in a pulp composed of solid phases of the ore suspended in a liquid phase which is a saturated solution of the ore, returning the liquid phase to the process for reuse in flotation at said controlled temperature, and reducing the temperature of said circulating saturated solution containing solid ore constituents thereby enriching the potassium chloride solids content thereof by deposition of potassium chloride out of said liquid phase in solid form.

25 30 23. In a cyclic froth flotation process for the treatment of sylvinitic ore, subjecting the ore to froth flotation at a substantially uniform temperature in a pulp composed of solid phases of the ore suspended in a liquid phase which is a saturated solution of the ore, returning the liquid phase to the process for reuse in flotation at said controlled temperature, and subjecting said circulating pulp as a preliminary to its use in flotation, to an artificial transfer of heat to compensate for its change in temperature occasioned in the cyclic movement.

ARTHUR J. WEINIG.